

Aug. 2, 1949.

C. C. WILSON ET AL

2,477,675

NONWOVEN FABRIC AND METHOD FOR MAKING SAME

Filed Nov. 18, 1947

4 Sheets-Sheet 1



Aug. 2, 1949.

C. C. WILSON ET AL

2,477,675

## NONWOVEN FABRIC AND METHOD FOR MAKING SAME

Filed Nov. 18, 1947

4 Sheets-Sheet 2



Charles C. Wilson,  
Herschel H. Cudd and  
Denzil V. Probasco

By Cushman, Darby & Cushman  
Attorneys

Aug. 2, 1949.

C. C. WILSON ET AL

2,477,675

NONWOVEN FABRIC AND METHOD FOR MAKING SAME

Filed Nov. 18, 1947

4 Sheets-Sheet 3



Inventors  
Charles C. Wilson,  
Herschel H. Cudd and  
Denzil V. Probasco

By  
Cushman, Darby & Cushman  
Attorneys

Aug. 2, 1949.

C. C. WILSON ET AL

2,477,675

NONWOVEN FABRIC AND METHOD FOR MAKING SAME

Filed Nov. 18, 1947

4 Sheets-Sheet 4

Fig. 6



Fig. 7



Fig. 8



Fig. 9



Fig. 10



Inventors

Charles C. Wilson,  
Herschel H. Cudd and  
Denzil V. Probasco

By  
Cushman, Darby & Cushman  
Attorneys

Patented Aug. 2, 1949

2,477,675

**UNITED STATES PATENT OFFICE**

2,477,675

## NONWOVEN FABRIC AND METHOD FOR MAKING SAME

Charles C. Wilson, Lanett, Ala., and Herschel H. Cudd and Denzil V. Probasco, West Point, Ga., assignors to West Point Manufacturing Company, West Point, Ga., a corporation of Alabama

**Application November 18, 1947. Serial No. 786,662**

**9 Claims. (Cl. 154—33)**

1

This invention relates to unwoven fabrics; a method of forming such fabrics, and equipment for practicing the method and producing the fabrics.

Unwoven fabrics are broadly old, but the methods and equipment heretofore used have not produced fabric of satisfactory make-up insofar as uniformity of fabric texture and strength in all directions are concerned.

Fabrics of this type are formed by depositing fibers drawn from any suitable source, such as a hopper, a card, or a doffer, in random fashion on a suitable foraminous receiving member in closely interlaced relation, the object being to secure textural uniformity and strength in all directions. Satisfactory results cannot, however, be obtained without particular attention to the removal of the fibers from the source; their distribution on the receiving member, and, as it is preferable in many cases, subjecting the web thus formed to a bonding treatment to stabilize the fibers and produce a web of proper density, uniformity, and stability, insofar as fiber relations are concerned.

In unwoven webs of the prior art, the fibers have been in some instances so laid as to parallel them either warpwise or fillingwise, resulting in a fabric of unequal strength in different directions as distinguished from the fabric of the present invention, in which the fibers are disposed in uniformly random fashion, free from knots or tangles, so that textural uniformity in all directions results.

It has been proposed in earlier methods to subject fibers to air currents in disposing them on a receiving surface, but such methods lack the technical efficiency of the present method, which involves the removal of the fibers directly from the supply by positive and direct air currents regulated within suitable ranges, insofar as intensity of flow is concerned, critical flow intensities being determined by the particular conditions met.

In practicing the invention herein disclosed, it has been found that the speed of the fiber carrying instrumentality which, in the present disclosure, is a doffer, must be considerably increased over the normal speeds in equipment of this kind as heretofore developed, the reason for this increased speed being that the fibers will be more completely and uniformly separated on the doffer and the knots and tangles straightened out, so that delivery from the fiber-carrying instrumentality to the fiber-receiving and web-forming instrumentalities results in a web of more uniform density and strength than under the slow speed equipment heretofore used.

Following fiber removal from the doffer, which is here shown as the source of the raw material, by air currents, such fibers, in suspended condition and in free relation to one another, are car-

2

ried at high speed through a fiber transfer duct which leads to a movable fiber receiving member, here shown as a screen cylinder, upon which the fibers are laid in random fashion and in closely matted relation. The thickness of the web, following the method and using the equipment hereinabove described, may be readily varied by regulating the speed of the movable fiber-receiving members so as to permit greater or less amounts of fiber to be deposited in a given period of time. Further, the width of the webs formed on the receiving surface may be varied so as to form a web of a width equal to the full length of the fiber receiving member, or fibers may be deposited on the receiving member in less than the full length of that member so as to form narrow webs or slivers. As stated, the present disclosure shows the removal of fibers directly from a doffer by air currents, the doffer being supplied in the usual manner from a card, but it will be understood that the removal of the fibers may be made directly from the card cylinder or other suitable source without the interposition of a doffer if desired.

25 In the description which follows, the method of producing the web is set forth in detail and the equipment for carrying out the method is illustrated in the drawings forming part of this disclosure. It is to be understood that this disclosure is illustrative and not restrictive as obvious variations from this disclosure within the scope of the invention may be made.

In the drawings:

Figure 1 is a view in side elevation showing the feed-in roller, the card, the doffer, the duct for removing the fiber from the doffer, and the fiber-receiving and web-forming screen.

Figure 2 is a sectional view of the equipment shown in Figure 1 with the web bonding instrumentalities and the web drying equipment added.

Figure 3 is a view in plan showing the doffer, the duct, the fiber-receiving screen, the spraying chamber, and the web-receiving roller, the driving gears for operating the parts being shown.

45 Figure 4 is an enlarged detail view, substantially on the line 4—4 of Figure 3, showing a portion of the doffer, the air duct which removes the fibers from the doffer, and the screen cylinder to  
50 which the fibers are delivered and on which the web is formed.

Figure 5 is a longitudinal sectional view of the web-forming screen on substantially the line 5-5 of Figure 4.

55 Figure 6 is a cross sectional view on substantially the line 6-6 of Figure 5.

Figure 7 is a detail view showing the end of the screen housing.

Figure 9 is a sectional view substantially on the line 9—9 of Figure 4.

Figure 10 is a view substantially on the line 10—10 of Figure 4.

Figure 11 is a detail view substantially on the line 11—11 of Figure 9.

Referring to the drawings by numbers, the same numbers designating the same parts in the several views, and considering first the disclosures in Figures 1 and 2, the frame 10, of any suitable or usual construction, carries the lap 11, the feed roller 12, the taker-in 16, and the card cylinder 17, as in the usual carding engine construction. These parts are all driven from any suitable source of power, a motor 18 being here shown from which power is supplied to drive the various instrumentalities through suitable belting and gears. This being the usual construction of carding engines, further detailed description of it is not necessary.

Adjacent the card cylinder 17 is a doffer 20, this doffer being driven from the card cylinder by means of the cross belt 21, the pulley 22, and the doffer belt 23, so as to revolve the doffer in the direction of the arrow opposite from the direction of rotation of the card cylinder 17. In the ordinary carding engine, the doffer rotates at a speed which is normally from 3 to 18 R. P. M., thus producing an attenuation or draft from 90 to 140 on the stock, with draft being defined as the peripheral speed of the doffer divided by the peripheral speed of the feed-in roll. In carrying out the present method, however, it has been found that the speed of the doffer must be higher relative to the speed of the feed-in roll and the card cylinder, and drafts from 500 to 1500 are necessary, a mean of 980 having been found to be a satisfactory draft, although it will be understood that the draft may be varied to some extent from the preferable mean. As a result of this range of high drafts, the card cylinder deposits the fibers on the doffer in a completely separated condition with each fiber being separate from the others and not gathered together in groups, bunches, or clumps of many fibers as are ordinarily present in equipment of this character when low speed doffing instrumentalities are used, so the fibers are laid on the doffer in an evenly distributed, well separated manner.

On the side of the doffer opposite its contact point with the card is provided a fiber transfer air duct 25, preferably of uniform dimension throughout its length, the doffer end of the duct 25 being placed in close relation to the teeth of the doffer and preferably the duct 25 will be slightly above the horizontal center of the doffer roll, as shown in Figure 2. It is desirable that the duct 25 which constitutes a confined uninterrupted path be of equal area in cross section throughout its length in order that there may be a uniform and even flow of air and fiber through the duct and turbulence caused by cross currents or swirls which might affect proper transmission of the fibers through the duct if it was of varying cross section, are avoided. The duct 25 may be provided, preferably on its upper side, with an air inlet 26, which inlet may be regulated by means of a gate 27 adjusted in any suitable manner as by the adjusting screw 28, so as to vary the size of the inlet 26 as may be desired. The duct 25 may be constructed in any suitable manner and is supported by means of a frame 29 secured to supporting side plates 30 mounted at one end on

the doffer frame and at the other end on the screen housing, presently to be described. The duct supporting frame 29 may be provided with transparent panels 31, preferably at its upper side in order that the flow of fiber through the duct may be observed and, if necessary, regulated by adjustment of the air inlet.

The delivery end of the duct 25 passes through a housing 32 having upper and lower sections in which is mounted a foraminous receiving surface, here shown as a revolving cylindrical screen 33 to which the duct delivers, the screen 33 being mounted to revolve on a fixed shaft 34. Screen 33 is driven by a pinion 35 carried on the shaft of gear 36, which gear 36 engages gear teeth on the screen cylinder, as shown in Figure 1. Gear 36 is driven by the gear 37 on pulley 38 belted by belt 39 to a gear assembly 40 driven from the motor 41. The gear assembly 40 is made up of a gear box having provision for interchanging the gears to vary speeds in the usual manner of changeable speed gear boxes. Interiorly of the screen 33 is a fixed shield 42 supported by shaft 34 and having an air-receiving opening 43 in line with the delivery end of the duct 25, as shown in Figure 4, and through which opening 43 the blast of air passes after it has deposited the fibers on the screen 33. The fixed shield 42 prevents any disturbance of the web laid upon the screen, the air being drawn out of the shield through exhaust connections 44 which open at their upper ends into the shield and the lower ends of which engage a fan casing 45 having a fan 46, conventionally shown, which fan is driven from any suitable source of power and creates a strong suction through the escape passage 44; the duct 25, and the air inlet 26. The air current created by the fan strips the fibers directly from the doffer 20, the usual doffer comb being dispensed with, and carries them in suspended and separated condition through the duct and deposits them on the screen 33. The speed of rotation of the screen may be varied through the change gear box or assembly 40 so as to give different screen speeds. By varying the speed of the screen, the thickness of the web formed by the fibers deposited on the screen may be widely varied. If a thin web is desired, the screen cylinder will be revolved at relatively high speed so that a thin layer of fibers is deposited on it. If a thicker web is desired, the speed of the screen may be slowed down and a thicker web results.

The delivery end of the duct 25 will be sealed off from the screen in any suitable manner as for example, by the flexible seals 47, as shown in Figure 4, or by means of the sealing off roller 48, which sealing off roller is mounted for free revolution by reason of its contact with the screen surface, this roller being preferably mounted in an adjustable spring mounting 49, as shown in Figures 9 and 11, so that its tension against the screen surface may be varied.

The screen 33, which is mounted to revolve on the fixed shaft 34, is carried by the spokes 50 mounted on the hub 51 and driven by the gear 36. It is essential that the screen be sealed off from the housing against the entry of air and this is accomplished, as shown in Figure 5, by providing sealing strips 52 carried by the housing 32, these strips effectually preventing the entrance of air to the interior of the screen.

The shield 42 is supported by the spokes 53 carried by the hub 54 which is pinned to the shaft 34 so as to hold the shield 42 in fixed posi-

tion. The shield 42 is sealed off at its ends from the screen 33 by the sealing strips 55 so as to confine the suction through the shield and permit its escape only through the connections 44.

In the form of the invention shown in Figure 1, the machine is set to form a narrow fabric or sliver, which sliver is doffed from the revolving screen 33 by means of a doffing roll 56, as shown in Figure 1, driven from pinion 35, from which doffing roll it passes to the drawing-off rolls 57 driven from any suitable source, and then passes to a sliver-receiving head 58, from which it is deposited in a sliver can 59.

In Figure 2, the machine is shown with means for bonding the web with any suitable bonding solution. Any convenient or desired bonding equipment can be used. As here shown, it comprises a supporting stand 60 having at its upper end a housing 61 in which are disposed spray heads connected to a pipe 62, which pipe may be supplied from any suitable source with the bonding solution. The web will be removed from the screen cylinder 33 and brought to the bonding area by a belt 63 mounted on rollers driven from any suitable source of power, so that, as the belt is driven, the web will be carried forward to drying instrumentalities hereinafter described. The belt may be formed of any suitable flexible and porous material such as cloth, woven wire, and the like. Any suitable means such, for example, as suction tube 65 may be provided to draw the bonding solution through and thoroughly impregnate the web. Any excess solution from the belt 63 will be caught by a drainage shelf 63' having a discharge tube 64' through which excess solution or overflow from the belt 63 will be delivered to any suitable receptacle.

The web passes from the belt 63 to drying and curing means as shown in Figure 2. This drying and curing equipment may be made up in different ways, but is here shown as an electrical dryer. It comprises a stand 66 having a heated box 67 in which is mounted for rotation rollers 68 having a carrier belt 69 to which the web is delivered from the belt 63. Heating and drying elements 70, conventionally shown as electrical heating elements to which current is supplied from any suitable source, are disposed above and below the belt 69 so that the web is subjected to complete drying and curing and then passes over a roller 71 and is delivered in bonded and dried condition.

Following the method and using the equipment herein shown and described, a non-woven fabric characterized by uniform density and texture and of equal strength in all directions, free from imperfections caused by knots and tangles, and of superior appearance may be produced.

Such variations from the specific construction here shown and described as involve only mechanical skill and are comprehended by the appended claims are to be regarded as within the range of the invention.

We claim:

1. The method of forming non-woven fabrics which comprises carding fibres and thus continuously providing a source of fibre supply of carded fibres, continuously delivering the said carded fibres from a supply to a foraminous fibre receiving member to form on such member a web, said delivery being accomplished by passing the carded fibres from said supply to the foraminous member by means of an air current through a confined uninterrupted path of equal area in cross section throughout its length, the fibres being

suspended in said air current during travel in said path to the foraminous fibre receiving member, forming a web on said member, and removing the web from said member.

- 5 2. The method of forming non-woven fabrics which comprises carding fibres and thus continuously providing a source of fibre supply of carded fibres, continuously delivering the said carded fibres from a supply to a foraminous fibre receiving member to form on such member a web, said delivery being accomplished by passing the carded fibres from said supply to the foraminous member by means of an air current through a confined uninterrupted path of equal area in cross section throughout its length, the fibres being suspended in said air current during travel in said path to the foraminous fibre receiving member, forming a web on said member, removing the web from said member, and bonding the web.
- 10 3. The method of forming non-woven fabrics which comprises carding fibres and thus continuously providing a source of fibre supply of carded fibres, continuously delivering the said carded fibres from a supply to a foraminous fibre receiving member to form on such member a web, said delivery being accomplished by passing the carded fibres from said supply to the foraminous member by means of an air current through a confined uninterrupted path of equal area in cross section throughout its length, the fibres being suspended in said air current during travel in said path to the foraminous fibre receiving member, forming a web on said member, removing the web from said member, bonding the web, and drying the web.
- 15 4. The method of forming a fibrous web which comprises carding fibres at a draft of at least 500 and thus continuously providing a source of fibre supply of carded fibres, continuously delivering said carded fibres from a supply to a foraminous fibre receiving member to form on such member a web, said delivery being accomplished by passing the carded fibres from said supply to the foraminous member by means of an air current
- 20 25 30 35

- through a confined uninterrupted path, the fibres being suspended in said air current during travel in said path to the foraminous fibre receiving member, forming a web on said member, and removing the web from said member.
- 40 45 50 55
5. The method according to claim 4 wherein said path is of equal area in cross section throughout its length.

6. As a new article of manufacture a non-woven fabric formed of random laid fibres matted together in uniform relation and characterized by freedom from knots and tangles and of uniform density and strength in all directions, and prepared by the method of claim 1.

- 60 65 70
7. As a new article of manufacture a non-woven fabric formed of random laid fibres matted together in uniform relation and characterized by freedom from knots and tangles and of uniform density and strength in all directions, and prepared by the method of claim 2.

8. As a new article of manufacture a non-woven fabric formed of random laid fibres matted together in uniform relation and characterized by freedom from knots and tangles and of uniform density and strength in all directions, and prepared by the method of claim 3.

9. As a new article of manufacture a non-woven fabric formed of random laid fibres matted together in uniform relation and characterized by freedom from knots and tangles and of uni-
- 75

form density and strength in all directions, and  
prepared by the method of claim 4.

CHARLES C. WILSON.  
HERSCHEL H. CUDD.  
DENZIL V. PROBASCO.

Number  
2,001,687  
2,146,698  
2,244,544  
5 2,396,178

| Name   | Date         |
|--------|--------------|
| Moss   | May 14, 1935 |
| Rogers | Feb. 7, 1939 |
| Smith  | June 3, 1941 |
| Kane   | Mar. 5, 1946 |

## FOREIGN PATENTS

| Country       | Date          |
|---------------|---------------|
| Great Britain | June 19, 1924 |
| Great Britain | Aug. 14, 1924 |
| Great Britain | June 5, 1942  |

## REFERENCES CITED

The following references are of record in the  
file of this patent:

## UNITED STATES PATENTS

Number  
217,476  
10 220,149  
545,638

| Number    | Name     | Date          |
|-----------|----------|---------------|
| 1,710,977 | Herbener | Apr. 30, 1929 |